

April 11, 1933.

C. LOCREILLE

1,903,718

PROCESS AND APPARATUS FOR PRINTING GLASS SHEETS

Filed March 27, 1930



C. Locreille  
INVENTOR

By: Marks & Clark  
Attn:

## UNITED STATES PATENT OFFICE

CLAUDE LOCREILLE, OF FAUQUEZ, BELGIUM

## PROCESS AND APPARATUS FOR PRINTING GLASS SHEETS

Application filed March 27, 1930, Serial No. 439,516, and in Belgium March 28, 1929.

Glass sheets which are to be decorated on one side with an embossed pattern or with a more or less deep impression are usually obtained by passing under a printing roll a sheet of cast or rolled glass which then is received on a table and is carried into the annealing furnace, its decorated side facing upwards. By its contact with the receiving table and the sole of the furnace the smooth 10 lower side of the sheet loses its evenness and the dust or even the grain of the materials forming said table and sole form therein small marks or blemishes, while the patterns on the upper side which is directly exposed 15 to the high temperature in the annealing furnace, are reburnt and lose their clearness.

The present invention is intended to obviate these inconveniences. According to this invention, instead of feeding the glass 20 sheet on the table and into the furnace with its printed side turned upwards, I feed the glass in such manner that the printed side is turned downwards and comes into contact with the receiving table and with the furnace 25 sole, the smooth side of the glass facing upwards. In this manner the smooth side does not suffer from the contact with the table and the sole, and I have found that it acquires in the furnace a high degree of polish, which 30 is very desirable, while the printed side sliding on the table and the sole, is less likely to be damaged thereby owing to the fact that air can circulate in its depressions and cavities, this side thus cooling more rapidly and hardening before any blemishes or blurring of 35 the pattern might be produced.

In carrying out my improved process the sheet is fed under the printing roll as usual and then turned before it is received on the 40 table so that its printed side comes to rest on the table as in the first case.

In carrying out this process I may use glass rolling trains of known types, with certain modifications which will be better understood with reference to the accompanying drawing in which I have illustrated by way of example an embodiment of my invention, the figure being a diagrammatic side 45 view of a rolling train in which the glass is fed over the printing roll.

In the drawing the rolling train comprises as usual two pressing rolls *a*, *b* and two drawing rolls *c*, *d*, one of which, *c*, is the printing roll provided on its surface with the pattern to be impressed into the glass. 55

As shown the printing roll *c* is located, as usual, above the smooth roll *d* and it impresses the pattern into the upper side of the glass sheet *e*. However, before said sheet comes to rest on the receiving table *f* it is turned around the roll *d* so that its smooth side comes on top and its printed side faces downwards. This arrangement offers the advantage that no particular construction is necessary in order to allow of replacing the printing roll. It is only required to reverse the position of the rolling train with respect to the entrance of the furnace and to reverse the direction of motion of the receiving table. The guiding plate *i* may be either spaced 60 away from the roll *d* sufficiently to allow of the sheet glass passing therebetween, or it may be in the form of a curved guide as shown. 65

The process described is also suitable for the production of "hammered" or so called "cathedral" glass. The roll *c* then has only very shallow irregular depressions and projections which are impressed on the side of the glass which comes into contact with the receiving table. Such contact cools the printed side of the glass which contracts, thus accentuating the "hammered" effect and imparting thereto a natural appearance. 75

The process according to this invention may of course be applied to other glass articles such as continuous strips of glass, and the arrangement of the apparatus described may be varied without departing from the scope of my invention as defined by the appended claims. 80

I claim:

1. In a process of printing glass sheets, rolling a sheet of glass in a plastic condition, feeding said sheet between an upper printing roll and a lower smooth roll, turning said sheet through an angle of more than 90° around the smooth roll so that its impressed side faces downwards and receiving said sheet on a supporting surface. 95
- 100

2. In apparatus for printing glass sheets, the combination of a glass rolling train, an annealing furnace, a movable table, a track for said table extending from under said 5 rolling train to said annealing furnace, said glass rolling train comprising an upper pair of rolls and a lower pair of rolls, said lower pair comprising an upper printing roll and a lower smooth roll, and means for guiding 10 a sheet of glass from said rolling train to said table through an angle of more than  $90^\circ$  whereby one side of the sheet will successively come into contact with said printing roll and with said table.
- 15 3. In apparatus for printing glass sheets, the combination of a glass rolling train, an annealing furnace, a movable table, a track for said table extending from under said rolling train to said annealing furnace, said 20 glass rolling train comprising an upper pair of rolls and a lower pair of rolls, said upper pair of rolls being nearer said furnace than said lower pair of rolls, said lower pair comprising an upper printing roll and a lower 25 smooth roll, and means for guiding a sheet of glass from under said printing roll around said smooth roll onto the table through an angle of more than  $90^\circ$  whereby the same side of the sheet successively comes into contact 3. with said printing roll and with said table.

CLAUDE LOCREUILLE.

35

40

45

50

55

60

65